

# UNITED STATES PATENT OFFICE.

RUSSELL S. PENNIMAN, OF JENKINTOWN, PENNSYLVANIA, ASSIGNOR OF  
ONE-HALF TO JOHN C. SCHRADER, OF MCCLAINSVILLE, NEW JERSEY.

## EXPLOSIVE COMPOUND.

SPECIFICATION forming part of Letters Patent No. 320,583, dated June 23, 1885.

Application filed May 3, 1883. (No specimens.)

*To all whom it may concern:*

Be it known that I, RUSSELL S. PENNIMAN, of Jenkintown, in the county of Montgomery and State of Pennsylvania, have invented certain new and useful Improvements in High Explosive Compounds; and I do hereby declare that the following specification is a true and exact description thereof.

In the new variety of high explosives hereinafter described I employ the nitrate of ammonia as an ingredient, and which substance, as is well known, furnishes a large quantity of gases when fired, but which has not heretofore been practically available as one of the constituents of high explosives, for the reason that no means, so far as I know, have been successfully devised to prevent its tendency to deliquesce in consequence of its natural affinity for moisture. To utilize this agent in an explosive, I superficially coat or envelop the particles of nitrate of ammonia, after they have been finely divided or brought to a granulated condition, with a fluid or viscous material, which will exclude them from contact with the atmosphere, and I prefer to make use for such envelope of the soft or viscous educts or products of petroleum, for the reason that petroleum or its products containing carbon, when applied in a fluid or viscous state to nitrate of ammonia, serves not only as a protector against deliquescence without impairing the granular or divided character of the nitrate, but also as a fuel to aid in the final explosion, and nitrate of ammonia thus coated with the soft or viscous educts or products of petroleum constitutes the subject of a separate application for Letters Patent, filed as a division hereof, Serial No. 113,217. My novel explosive compounds are produced by combining with the so-protected nitrate of ammonia any suitable detonating compound or explosive agent which, under proper conditions, will serve to fire the protected nitrate of ammonia.

In herein referring to detonating materials and compounds and to explosive agents I do not include detonating caps or fuses, but only such detonating materials or compounds as can be mixed or compounded with the protected nitrate.

My improved manufacture, hereinafter more fully described, constitutes an explosive compound of great power when confined and fired under suitable conditions, but which, under ordinary circumstances, and when subjected to the usual incidents of handling and transportation, is entirely harmless.

In order to carry out my invention to the best advantage, I take a quantity of the nitrate of ammonia of commerce in its usual solid or crystallized form and melt it at a temperature of, say, 320° Fahrenheit in a suitable vessel. The next step is to granulate the nitrate of ammonia so melted, and for this purpose it may be transferred to another kettle provided with a water-jacket, and be stirred continuously, while at the same time the heat of the water-jacket is allowed to be reduced steadily until the liquid nitrate of ammonia as the result of stirring and cooling has become granulated.

The process thus far is one which is known to chemists, and the above or any other preferred method may be employed for granulating the nitrate of ammonia.

The nitrate of ammonia having been granulated, the next step is to protect the granules from atmospheric contact, so as to prevent their deliquescence, and this I do by the use of the semi-fluid educts or products of petroleum or other equivalent substance which will form a soft or viscous envelope or coating for each of the granules of nitrate of ammonia and protect them from the influence of atmospheric moisture. I prefer to use the heavy educts or products of petroleum, but crude petroleum will answer the purpose very fairly. It is desirable, however, that the protecting material should have considerable consistency and be in the viscous or semi-fluid condition. To accomplish this protection of the nitrate of ammonia against the influence of atmospheric moisture, I thoroughly mix by stirring with any given quantity of nitrate of ammonia twelve per cent. (more or less) of its weight of such petroleum or its educts or products, enough of such protecting substance being used to completely coat the granules of the nitrate of ammonia, and the operation of stirring should be continued long enough to thor-

oughly accomplish this result, and if the quantity of protecting agent above specified is not sufficient more should be added.

Protected nitrate of ammonia, as above described, is now suitable to be combined with any detonating compound or substance which will when fired create a sufficient amount of heat to set fire to the nitrate of ammonia and form with the said nitrate of ammonia a high explosive, suitable when confined and fired to be used for blasting and similar purposes.

For a detonating material to be combined with the said protected nitrate of ammonia, I rely upon chlorate of potash, also mixed with a similar or the same soft or viscous protecting agent. I take, say, eighty-five parts, by weight, of chlorate of potash and add fifteen parts of the heavy hydrocarbon similar to that used in protecting the nitrate of ammonia, and thoroughly mix the two together in any of the ways usually practiced by any of the manufacturers of explosives. In place of this detonator other agents for the same purpose may be employed in combination with the protected nitrate of ammonia, provided that such detonators or explosives have sufficient strength and capacity to fire the nitrate of ammonia. I rely, however, upon the chlorate of potash, for the reason that it is not affected by extreme cold, and under all reasonable conditions of use is harmless. I now take equal parts, by weight, or thereabout, of the so-protected nitrate of ammonia and the chlorate of potash, treated as above, to form a detonator, and thoroughly mix the two substances in any convenient or preferred way.

The resulting article is a high explosive, which can be handled and transported with safety, and it can be subjected to percussion when unconfined without danger, or be subjected to the action of flame without any explosion. When, however, it is under confinement, as when used for blasting purposes, and fired by a detonating cap or a strong fuse, it is followed by the most destructive effects. The chlorate of potash sets fire to the protecting envelope which surrounds each particle of the granulated nitrate of ammonia, and this envelope, being a hydrocarbon, serves as a fuel to aid in firing the nitrate of ammonia and contributing gases to increase the effect of the explosion.

I am aware that deliquescent or hydroscopic nitrates have heretofore been employed with various ingredients in the manufacture of explosive compounds, and that such nitrates have been combined with such solid, fatty, or waxy bodies as paraffine, naphthaline, stearine, ozocerite, palmitate of cetyl, and hard pitch, and also that in some cases some of these last-named ingredients have been employed for obviating the deliquescent tendency of said nitrates; but so far as my knowledge extends, such solid, waxy, or fatty substances have

never heretofore been combined with said nitrates in their isolated condition, or employed while in a fluid, semi-fluid, or viscous state, to envelop the particles of the nitrate, as distinguished from being ground with the nitrates in connection with other ingredients, such as finely-powdered animal or vegetable charcoal, coal-dust, &c.

The order of steps hereinbefore stated for producing my improved high explosive is not the essence of the invention. The end to be accomplished is the production of a new variety of high explosives composed of nitrate of ammonia, protected, as described, by a fluid, semi-fluid, or viscous coating or envelope applied to the separate particles or granules of nitrate of ammonia to protect the same against deliquescence, and the chlorate of potash operating as a detonating or firing agent, the office of which, having been itself fired, by a detonating cup or fuse, is to fire the nitrate of ammonia under suitable conditions.

The proportion of the constituents named may be twelve and one-half parts of the fluid or viscous protecting material; forty-two and one-half parts of chlorate of potash, and forty-five parts of nitrate of ammonia; but these proportions may be varied to suit different conditions of use. In the preparation of the article a portion of the fluid, semi-fluid, or viscous protecting material may be mixed with the nitrate of ammonia, and the residue with the chlorate of potash, as hereinbefore described, or all of the protector may be mixed with the nitrate of ammonia and then this compound mixed with the chlorate of potash; or all of the protector may be mixed with the chlorate of potash, and then this compound mixed with the granulated nitrate of ammonia, it always being understood that enough of the protector be employed to thoroughly coat the individual granules of the nitrate of ammonia.

This explosive for immediate use may be compounded at all seasons regardless of temperature, but when manufactured and on storage or transportation, temperatures above, say, 80° Fahrenheit should be avoided because of a tendency to spontaneous combustion.

What I claim as my invention, and desire to secure by Letters Patent, is—

A high explosive composed of nitrate of ammonia in a finely divided or granulated condition, and protected from contact with the atmosphere by a fluid or viscous coating or envelope composed of petroleum or its soft educts or products, in combination with chlorate of potash operating as an explosive or detonator for firing the protected nitrate, substantially as specified.

RUSSELL S. PENNIMAN.

Witnesses:

C. MATHER,  
JOSEPH W. GRISCOM.